

# United States Patent [19]

Spiertz et al.

[11] 3,802,886

[45] Apr. 9, 1974

[54] **PHOTOSENSITIVE MATERIAL**

[75] Inventors: **Elisabeth Jacoba Spiertz; Leendert Klaas Hellinga Van Beek**, both of Emmasingel, Eindhoven, Netherlands

[73] Assignee: **U.S. Philips Corporation**, New York, N.Y.

[22] Filed: **Mar. 13, 1972**

[21] Appl. No.: **234,408**

**Related U.S. Application Data**

[63] Continuation of Ser. No. 865,958, Oct. 13, 1969, abandoned.

[30] **Foreign Application Priority Data**

Oct. 26, 1968 Netherlands ..... 6814762

[52] **U.S. Cl.** ..... **96/75, 96/36.2, 96/48 PD, 96/49, 96/86 R, 96/87 R, 96/91 R**

[51] **Int. Cl.** ..... **G03c 1/56, G03c 1/76**

[58] **Field of Search** ..... **96/48 PD, 49, 75, 91 R**

[56] **References Cited**

**UNITED STATES PATENTS**

2,657,137 10/1953 Kessels ..... 96/91 R

|           |         |                      |          |
|-----------|---------|----------------------|----------|
| 2,735,773 | 2/1956  | Dippel et al. ....   | 96/48 PD |
| 2,838,398 | 6/1958  | Dippel et al. ....   | 96/49    |
| 3,086,833 | 4/1963  | Streck.....          | 8/79     |
| 3,159,487 | 12/1964 | Kreiger et al. ....  | 96/75    |
| 3,390,998 | 7/1968  | Cole .....           | 96/48 PD |
| 3,409,438 | 11/1968 | Lokker .....         | 96/49    |
| 3,464,823 | 9/1969  | Halperin et al. .... | 96/49    |
| 3,506,442 | 4/1970  | Kerwin.....          | 96/41    |
| 3,615,560 | 10/1971 | Jonker et al. ....   | 96/75    |

**OTHER PUBLICATIONS**

Kosar, J., "Light-Sensitive Systems," Wiley & Sons, 1965, pp. 255, 292, 294 and 272-276.

*Primary Examiner*—Charles L. Bowers, Jr.  
*Attorney, Agent, or Firm*—Norman N. Spain; Frank R. Trifari

[57] **ABSTRACT**

A photosensitive layer capable of producing a physically developed contrast containing a significantly decreased number of pinholes in which a non-conducting support is provided with a photosensitive diazosulfonate, mercurous ion and/or silver ions and a saccharide having an aldehyde group.

**5 Claims, No Drawings**

## PHOTOSENSITIVE MATERIAL

This is a continuation, division, of application Ser. No. 865,958, filed Oct. 13, 1969 now abandoned.

The invention relates to photosensitive material comprising an at least superficially electrically non-conducting support in which or on which the actual photosensitive layer comprising a stable aromatic diazosulphonate is provided.

Known materials comprises as a photosensitive substance, an aromatic diazo compound, for example, a diazo thioether or a diazosulphonate or a diazocyanide. The action of these diazo compounds, when being used in photographic material, is based on the recognition that they yield an unstable intermediate product upon exposure, which can at least partially dissociate into diazonium ions and anions, in the abovementioned case alkyl thiolate, sulphite and cyanide, respectively. When an exposed layer comprising such a diazo compound is contacted with an aqueous solution containing mercurous ions and preferably also silver ions, a latent image is formed which consists of physically developable mercury or amalgam nuclei, because the said unstable intermediate products and/or the anions produced during dissociation are capable of withdrawing mercuric ions from the equilibrium:



which exists in a satisfactorily prepared solution of a mercurous salt. In an embodiment of the diazosulphonate material (Netherlands Pat. application 6,606,656) the mercurous salt and the silver salt are already present in the photosensitive layer, so that the said nucleation is directly set in during exposure in a layer which is not completely dry. The metal nuclei images formed are intensified by physical development to photographic metal images of the required blackening.

A diazosulphonate layer preferably comprises also a so-called anti-regression agent, which is a compound which, prior to the nucleation reaction having taken place, prevents the diazo compound from being reformed from its light reaction product by binding either the diazonium ion or the sulphite ion or both ions in such a manner that the sulphite ion retains the possibility to react with mercurous ions in the presence of moisture while forming mercury nuclei these anti-regression agents are described and a large number of them are listed in British Pat. 748,172, published Apr. 18, 1956.

The photosensitive layer may be obtained, for example, by saponification of a surface layer of a foil consisting of a cellulose ester, or by anodic oxidation of an aluminium foil succeeded by impregnation of the hydrophilic layer obtained with a solution comprising the photosensitive substance and possibly the auxiliary substances. It may alternatively comprise a larger or smaller part of a hydrophilic support, such as paper or cellophane. The material may furthermore consist of a support of dimensionally stable material which cannot be impregnated with water, and which is provided with a hydrophilic photosensitized layer.

It has been found that inhomogeneities in the photosensitive layer give rise to the formation of small holes of microscopic dimensions. Such inhomogeneities may occur, for example, when the diazo compounds are not homogeneously distributed in the layer. Much more important was the phenomenon that also the light reac-

tion product may cause deposit formation in the layer which in some known modifications is still advanced by the presence of metal ions which with the anions produced during exposure yield sparingly soluble salts.

Such inhomogeneities in the layer are insufficiently reactive at the nucleation reaction and probably cause the occurrence of small holes of microscopic dimensions in the developed image. The number of these holes was unfortunately found to be greatest in those photosensitive materials which due to their high resolving power might eminently be suitable for the manufacture of photomasks for integrated circuits. For such uses, however, the occurrence of large numbers of holes is unacceptable because these are transferred onto the used photosensitive etching resists and would therefore lead to a high percentage of rejects during manufacture. It is true that the number of holes can be reduced considerably by careful choice of the support material, because it has been found that plasticizers or impurities present in some foils or certain chemically active groups in the macromolecular base indirectly or directly cause holes. A further improvement may be obtained by working as carefully as possible and with the exclusion of dust during the manufacture of the foils. All these steps combined cannot, however, decrease the level of the number of holes per sq.cm any further than to several thousand, counted microscopically at an enlargement of 60 times in areas of blackening  $D = 3.5$ . This is, however, still unacceptable for the above-mentioned uses.

The material according to the invention provides a developed image which, in areas of blackening  $D = 3.5$  important for practice, has a number of holes per sq.cm as microscopically observed at an enlargement of 60 times which as a rule is considerably smaller than 1,000. It is characterized in that in addition to an aromatic diazosulphonate, an antiregression agent, and possibly buffers and/or mercurous ions and silver ions, the photosensitive layer comprises a saccharide having an aldehyde function.

Such a saccharide, which is preferred on account of its greatest activity, is maltose, since it gives a number of holes of far less than 1,000. In the embodiment in which mercurous and silver ions are present in the layer, maltose is preferably used in a molecular concentration which is at most one-fourth of that of diazosulphonate. Lactose, glucose, galactose and starch are also suitable, but they have a smaller activity than maltose. The presence of an aldehyde function in the molecule has been found to be essential: hence, saccharose does not show any effect at all.

According to a further elaboration of the invention it was found that an additional reduction of the number of holes is obtained when the solution by which the layer is photosensitized also comprises a non-ionic wetting agent in a concentration of at least 0.1 percent by weight.

The added saccharides and wetting agents probably enhance the distribution of the light reaction product in the layer so that the risk of the occurrence of concentration gradients and hence the possibility of deposit formation is reduced. There is evidence that the saccharides having an aldehyde function slightly bind the sulphite, although this is denied in literature (A.F. Holleman Leerboek der Organische Chemie 1960, pages 368 and 401, etc.). Maltose also shows the effect of slightly increasing the sensitivity.

The invention will now further be described with reference to the following examples.

1. Strips of cellulose triacetate foil, saponified up to a depth of 2  $\mu\text{m}$ , were unilaterally photosensitized by bathing them for 2 minutes in aqueous solutions containing per litre:

- a. 0.4 mol sodium salt of 4-methoxybenzenediazo-sulphonic acid, 0.1 mol cadmium lactate, 0.1 mol calcium lactate, and 0.1 mol lactic acid;
- a1. the same components as solution a + 0.2 mol glucose;
- a2. the same components as solution a + 0.2 mol maltose;
- b. the same components as solution a + 0.1 percent of Lissapol N (i.e. a non-ionic surface-active substance comprising a condensation product of alkyl phenols and ethylene oxide);
- b1. the same components as solution b + 0.2 mol maltose.

After removing the adhering liquid by wiping it off between two rubber strips, the strips were dried in a hot stream of air, and subsequently stored for approximately 12 hours in a space through which air of 50 percent relative humidity flows. After exposure of the strips with the aid of a sensitometer, a nuclei image was introduced by treatment for 4 seconds in a bath containing per litre of water 0.005 mol mercurous nitrate and 0.0066 mol silver nitrate, and 0.1 percent of Lissapol N. Subsequently the strips were rinsed for a short time in deionized water and developed for 4 minutes in a physical developer containing per litre of water: 0.05 mol. ferrous ammonium sulphate, 0.01 mol ferric nitrate, 0.1 mol citric acid, 0.2 g of Armac 12D, (i.e., a cationic surface-active substance which consists for approximately 90 percent of dodecylamine acetate, for 9 percent of tetradecylamine acetate and furthermore of higher alkylamine acetates) and 0.2 g of Lissapol N.

After rinsing in deionized water and drying, the sensitometer strips were measured with the aid of the sensitometer. In the area of density for visible light of  $D = 3.5$  the number of holes was counted at an enlargement of 60 times. The numbers found were multiplied by a constant factor in order to obtain numbers per sq.cm. The results were, for strips photosensitized with:

- solution a 2,600 per sq.cm:  $\log E = 5.34$
- solution a1 1,450 per sq.cm:  $\log E = 4.73$
- solution a2 550 per sq.cm:  $\log E = 4.72$
- solution b 1,500 per sq.cm:  $\log E = 5.10$
- solution b1 550 per sq.cm:  $\log E = 4.67$

The exposure energies E are expressed in ergs/sq.cm.

2. Strips of saponified carrier material of Example 1 were photosensitized with solutions containing per litre of water:

- a. 0.2 mol cadmium salt of 4-methoxybenzenediazo-sulphonic acid, 0.005 mol mercurous nitrate, 0.01 mol silver nitrate, 0.02 mol cadmium lactate and 0.1 percent of Lissapol N;

a1. the same components as  $a = 0.2$  mol glucose;

a2. the same components as  $a = 0.01$  mol maltose.

After sensitometric exposure, a nuclei image was introduced by treatment for 4 seconds in a bath containing per litre of water 0.005 mol mercurous nitrate, 0.0025 mol silver nitrate, and 0.1 percent of Lissapol N. Subsequently the strips were rinsed for 4 seconds in deionized water and developed as described under 1. The results were, for strips photosensitized with:

Solution a: 2,500 per sq.cm  $\log E = 4.90$

Solution a1: 1,900 per sq.cm  $\log E = 4.97$

Solution a2: 750 per sq.cm  $\log E = 4.68$ .

What is claimed is:

1. A photosensitive material suitable for physical development comprising a support having a surface which is essentially electrically non-conductive, the surface having a photosensitive layer which contains a stable aromatic diazo-N-sulfonate, at least one saccharide containing an aldehyde moiety selected from the group consisting of maltose, lactose, glucose, galactose and starch and an antiregression agent for the diazosulfonate.

2. The photosensitive material of claim 1 wherein in addition silver and mercurous salts are present in the photosensitive layer.

3. The photosensitive material of claim 1 wherein the saccharide is present in a molecular concentration that is not greater than one-fourth of that of the diazosulfonate.

4. The photosensitive material of claim 3 wherein the saccharide is maltose.

5. The photosensitive material of claim 4 wherein a nonionic wetting agent is present in the photosensitive layer.

\* \* \* \* \*

UNITED STATES PATENT OFFICE  
CERTIFICATE OF CORRECTION

Patent No. 3,802,886

Dated April 9, 1974

Inventor(s) ELISABETH JACOBA SPIERTZ ET AL

It is certified that error appears in the above-identified patent and that said Letters Patent are hereby corrected as shown below:

In the Title page:

[30] "Oct.26,1968" should be -- Oct. 16,1968 --.

Signed and sealed this 10th day of September 1974.

(SEAL)

Attest:

McCoy M. GIBSON, JR.  
Attesting Officer

C. MARSHALL DANN  
Commissioner of Patents